

Patented May 11, 1926.

1,583,801

# UNITED STATES PATENT OFFICE.

OTTO SCHMIDT, OF LUDWIGSHAFEN-ON-THE-RHINE, GERMANY, ASSIGNOR TO  
BADISCHE ANILIN- & SODA-FABRIK, OF LUDWIGSHAFEN-ON-THE-RHINE, GER-  
MANY, A CORPORATION OF GERMANY.

## ARTIFICIAL TANNING SUBSTANCE.

No Drawing.

Application filed August 24, 1925. Serial No. 52,233.

This present invention relates to improvements in the preparation of artificial tanning substances.

It is already known that by treating charred vegetable materials such as charcoal with nitric acid or nitrogen oxids substances possessing tanning properties are obtained.

I have now found that the tanning properties of these substances are much improved by bringing them into a weakly acid condition. This result may be obtained by neutralizing them partially or wholly and again slightly acidulating them. Preferably, the products are neutralized to about 20 to 40 per cent; any other degree of neutralization, however, may also be suitable.

When tanning substances prepared according to this invention are used the advantage that the hides do not swell too much from the commencement of the operation results and the tanning process is thereby accelerated and the hides tanned more thoroughly. The color of the leather is also better and lighter by reason of the hides not

swelling so much as aforesaid.

I have further found that especially good tanning substances are obtained by oxidizing charcoal containing an unusual quantity of oxygen compounds and then partially neutralizing the product. Such charcoals as contain 9 per cent or more of oxygen, calculated on the coaly substance free from ashes, are especially suitable, yielding with a moderate consumption of nitric acid or nitrogen oxids tanning substances of a remarkably light color. It is generally sufficient to neutralize a small fraction of the acidity of the product.

The said substances can be mixed, before or after reducing their acidity, with other artificial tanning substances, such for example as formaldehyde-naphthalene-sulfonic acid condensation products or their salts, or other artificial tanning substances containing one or several sulfonic acid groups, or their salts. They can also be mixed with vegetable tanning substances such, for example, as quebracho and the like. With such a combination, and especially that with vegetable tanning matters, the grain of the leather will keep much better than in the case of leather tanned by mixtures with the raw oxidation products pos-

sessing no reduced acidity; in the latter case the grain is often brittle.

The nature of this invention is more fully explained by the following examples to which however the invention is not restricted. The parts are by weight.

### Example 1.

20 parts of a dry tanning substance, obtained by oxidizing charcoal with nitric acid, possessing an acidity equal to about 10 cubic centimetres of normal caustic soda liquor to 1 gram of the substance, are dissolved in 80 parts of water and mixed with 40 parts of normal caustic soda.

280 parts of the tanning solution so prepared are diluted with water to 1000 parts by volume. Into this tanning bath 60 parts of well delimited hide are introduced. The hide is tanned in the course of 8 to 10 days and a full, soft leather of a red-brown color is obtained.

### Example 2.

140 parts by weight of the solution prepared as described in the first paragraph of Example 1 are mixed with 80 parts of chestnut-wood extract and then diluted with water to 1000 parts by volume. About 60 parts of carefully delimited hide are tanned in this bath in the usual manner in 10 to 14 days. A light-brown full leather with stable grains is obtained.

The tanning oxidation product may be prepared as follows: 100 parts of finely powdered charcoal with an oxygen content of 14.8 per cent, calculated on ash-free substance, are stirred with 160 parts of water. 120 parts of a 95 per cent nitric acid solution are then slowly added whereupon the mass is slowly heated to the boil. After boiling for 12 hours the greater part of the liquid is distilled off and 680 more parts of a 95 per cent nitric acid solution are added while continuing boiling for two days. The main part of the aqueous nitric acid left in the vessel is distilled off, employing finally a vacuum, and for removing the last traces of nitric acid an addition of water is made repeatedly with subsequent evaporation.

The residue is powdered, giving an orange to yellowish powder which is completely soluble in water and has excellent tanning

properties. Instead of nitric acid, nitrogen oxide may be employed.

I claim:

- 5 1. As an article of manufacture an oxidation product of charcoal possessing tanning properties and being partly in the form of an acid and partly in the form of a soluble salt.
- 10 2. As an article of manufacture an oxidation product of charcoal possessing tanning properties and being partly in the form of an acid and partly in the form of a soluble salt in combination with another tanning material.
- 15 3. The process of producing tanning materials which consists in acting on charcoal with a nitric acid solution and partly neutralizing the oxidation product with a base forming a soluble salt.

4. The process of producing tanning materials which consists in oxidizing a charcoal containing at least 9 per cent of oxygen, calculated on the coaly substance free from ashes with nitric acid and partly neutralizing the oxidation product with a base forming a soluble salt. 20

5. The process of producing tanning materials which consists in oxidizing a charcoal containing at least 9 per cent of oxygen, calculated on the coaly substance free from 25 ashes with nitric acid, partly neutralizing the oxidation product with a base forming a soluble salt, and mixing the product with a natural tanning extract. 30

In testimony whereof I have hereunto set 35 my hand.

OTTO SCHMIDT.